

# UNITED STATES PATENT OFFICE.

LOUIS FRANÇOIS PARIS, OF PARIS, FRANCE.

## PROCESS FOR SECRETING FUR AND HAIR.

1,213,403.

Specification of Letters Patent.

Patented Jan. 23, 1917.

No Drawing. Application filed March 3, 1914, Serial No. 822,179. Renewed June 20, 1916. Serial No. 104,804.

To all whom it may concern:

Be it known that I, LOUIS FRANÇOIS PARIS, citizen of the Republic of France, residing at 28 Rue de Constantinople, Paris, in the Republic of France, have invented new and useful Improvements in Processes for Secreting Fur and Hair, of which the following is a specification.

This invention relates to a process for secreting hair intended for the manufacture of felt, without using mercury.

According to this invention the secreting is obtained by the action in a cold state or in a drying oven of compounds that are formed when the following substances are made to react on one another in water: nitric acid, hydrochloric acid, zinc chlorid, a metallic nitrite (preferably of sodium), a metallic hypochlorite (preferably of sodium). At the instant these substances are mixed simultaneous reactions are produced, that finally leave the double chlorid of nitrosyl and zinc in solution as well as a nitrous anhydrid and a small excess of nitric acid and hydrochloric acid. These reactions are as follows:

1. The hydrochloric acid reacts on the hypochlorid of sodium and produces free chlorin, sodium chlorid and water according to the formula:



2. The nascent chlorin reacts on the nitrogen bioxid produced by the decomposition of the nitrite of sodium and forms nitrosyl chlorid:



3. This latter compound combines with the zinc chlorid and produces a double chlorid of the formula:



the solution of which is stable in the medium used.

4. The nitrite of sodium is decomposed by the mixture of acids and produces neutral salts *i.e.* nitrate and chlorid of sodium while setting free nitrous anhydrid. A large part of the latter remains as a stable solution in the medium used, as will readily be seen by the intense bluish-green tint it gives to the liquid. A further part is decomposed by

the water and produces nitric acid and nitrogen bioxid according to the formula:



The nitrogen bioxid that is thus formed reacts with the free chlorin under the conditions above referred to and produces nitrosyl chlorid.

In order to give the hair treated a glossy appearance and protect the hides against the damages produced by mites, a certain quantity of a neutral salt is added to the mixture, that has just been referred to. This salt, which may be of any kind, covers each hair, when the latter is dried, with a thin brilliant pellicule that secures the conservation of the hair. A barium or strontium salt is preferably used to precipitate as an insoluble sulfate the free or combined sulfuric acid which occurs owing to the use of impure commercial products. This impurity has indeed the serious drawback of slightly parchmentizing the hides and thus rendering difficult the subsequent use of the so called vermicelli for the manufacture of glue.

The activity of the secreting solution is such that it allows of fulling the hat bells obtained with the hair prepared in this manner, without using sulfuric acid.

The proportions of the various substances used may vary within pretty large limits without substantially modifying the secreting properties.

The following examples contain the proportions that have allowed of obtaining the best results.

*Example I—Yellow secreting liquid.*—In 8 liters of cold water the following substances are made to dissolve: sodium nitrite, 300 gr.; strontium nitrate, 300 gr. When the solution is finished 100 cc. of hypochlorite of sodium (commercial solution) are added. The following mixture is then added slowly and while stirring gently, the said mixture being prepared at the moment it is to be used: nitric acid, 36°, 1800 cc.; hydrochloric acid, ord., 500 cc.; zinc chlorid, (sol. of 45°,) 350 cc. The brushing and stoving of the hides is made as in the case of mercury secreting liquid.

*Example II—Pale secreting liquid.*—In 8 liters of cold water are made to dissolve:

sodium nitrite, 10 gr.; strontium nitrate, 300 gr. When the solution is finished 100 cc. of sodium hypochlorite are added, whereupon the following mixture is slowly 5 poured into the solution while stirring gently: nitric acid, 36°, 500 cc.; hydrochloric acid, 1000 cc.; zinc chlorid, 45°, 350 cc.

The mixture must be prepared at the moment it is used. The brushing and drying 10 is made as in the case of mercury secreting liquid.

The same results are obtained with the yellow as well as with the pale secreting 15 liquid, if the hides are successively brushed with the separate solutions, the reactions being thus produced on the hair itself.

Having now described my invention, what I claim as new and desire to secure by Letters Patent is:

20. 1. A process for secreting hair intended for the manufacture of felt, which consists in subjecting the hair to the action of the compounds that arise when nitric acid, hydrochloric acid, zinc chlorid, sodium nitrite and sodium hypochlorite are made to react 25 in an aqueous solution.

2. A process for secreting hair intended for the manufacture of felt, which consists in subjecting the hair to the action of ni-

30 trous anhydrid, nitrosyl chlorid and a combination of the nitrosyl chlorid with a metallic chlorid.

3. A process for secreting hair intended for the manufacture of felt, which consists in subjecting the hair to the action of the 35 compounds that arise when nitric acid, hydrochloric acid, zinc chlorid, sodium nitrite and sodium hypochlorite are made to react in an aqueous solution to which a neutral salt has been added, substantially as de- 40 scribed and for the purpose set forth.

4. A process for secreting hair intended for the manufacture of felt, which consists in subjecting the hair to the action of the 45 compounds that arise when nitric acid, hydrochloric acid, zinc chlorid, sodium nitrite and sodium hypochlorite are made to react in an aqueous solution, to which a salt of an alkaline earth has been added, substantially as described and for the purpose set forth. 50

In testimony whereof I have signed my name to this specification in the presence of two subscribing witnesses.

LOUIS FRANÇOIS PARIS.

Witnesses:

ANTOINE LAVOIX,  
HANSON C. COXE.